

# UNITED STATES PATENT OFFICE.

JOHN WAFFEN, OF HANCOCK, MICHIGAN, ASSIGNOR TO HIMSELF, AND DANIEL KLOECKNER AND PHILIP SCHEUERMANN, BOTH OF SAME PLACE.

## DYNAMITE.

SPECIFICATION forming part of Letters Patent No. 398,559, dated February 26, 1889.

Application filed June 16, 1888. Serial No. 277,367. (No specimens.)

To all whom it may concern:

Be it known that I, JOHN WAFFEN, of Hancock, in the county of Houghton and State of Michigan, have invented a new and Improved Explosive Compound, of which the following is a full, clear, and exact description.

This invention consists of a new and useful composition of matter to be used as a high explosive.

10 The composition consists of two separately prepared mixtures or substances which are afterward mixed together and combined to form the explosive. The first of these mixtures constitutes a chemically-active absorbent, and the second one a specially-prepared

parts of nitro-glycerine proper and the six parts of collodion, gradually pouring the latter into the nitro-glycerine and stirring the mass while doing so, whereupon in a short interval of time the ingredients will be converted into the thick sirup-like mass above mentioned. By thus treating the nitro-glycerine a great transmutation is effected—that is to say, the danger attaching to ordinary nitro-glycerine is materially diminished, its celerity 55 augmented, and its explosive power multiplied—and such specially-prepared nitro-glycerine mixed with any absorbent will resist any pressure applied to cause its outflow or separation from the absorbent.

60 To produce a greater development of gases and to retard the suddenness of the action of the explosive, the chemically-active absorbent hereinbefore described has been designed. This chemically-active absorbent is in itself 70 highly inflammable. By the combination of the picric acid, sulphur, and decayed wood with the nitrate of soda the volume of gases resulting from the preparation is materially augmented and secures the perfect combustion of the nitro-glycerine when mixed with it, while the carbonate of soda in the composition is specially designed to prevent that spontaneous explosion which is of such frequent occurrence with nitro-glycerine compounds as ordinarily prepared.

65 The first part of the composition—that is, the chemically-active absorbent—has its several ingredients ground and mixed by any suitable apparatus, but preferably by putting them, together with balls made of wood or copper, into a horizontally-rotating wooden cylinder, said balls being of about one-third greater weight than the quantity of the above-named composition in the cylinder, which is kept revolving for about eight hours (more or less) at a speed not exceeding twenty-four revolutions, or thereabout, per minute. The chemically-active absorbent having had its ingredients thus or otherwise suitably ground and mixed, I then proceed to add the specially prepared nitro-glycerine, which consists of

75 ninety-four per cent. of nitro-glycerine proper and six per cent. of collodion, the collodion having the property of converting the nitro-glycerine into a thick sirup-like fluid. To 85 prepare this nitro-glycerine I put into a wooden vat of suitable size the ninety-four parts of the prepared chemically-active absorbent, and placing it in a wooden vessel; gradually add thereto about forty parts of the prepared nitro-glycerine compound and mix the whole thoroughly until the entire mass shall present the appearance of a uniformly fatty substance, which completes the 90 production of the explosive. Such explosive may then be placed in cylindrical-shaped paper cartridges, which may be packed in wooden boxes ready for use. The appearance of the explosive is that of a dark-brown 95 plastic mass, and its properties are such that it will ignite rapidly upon the application of fire without causing any explosion; but by the use of the percussion-cap and fuse employed for exploding other preparations of 100 nitro-glycerine a loud detonation will be pro-

duced. Said explosive is not affected by water or moisture, and is not susceptible of change excepting when exposed to a temperature exceeding 110° Fahrenheit. An explosion, however, may be produced by violent impact with or blow on it of iron, steel, or other hard substance.

To prevent accident, the same precaution should be used in handling this explosive as is or should be observed in using and handling all high explosives or combinations of nitro-glycerine.

Having thus described my invention, what I

claim as new, and desire to secure by Letters Patent, is—

The herein-described composition of matter to be used as an explosive, consisting of nitrate of soda, decayed wood, picric acid, sulphur, carbonate of soda, and nitro-glycerine having collodion mixed with it, substantially as and in or about the proportions specified.

JOHN WAFFEN.

Witnesses:

JOSEPH A. CROWELL,  
G. KLOECKNER.